

# UNITED STATES PATENT OFFICE.

ALCAN HIRSCH AND MARX HIRSCH, OF NEW YORK, N. Y.

## FLOTATION AGENT AND METHOD OF MAKING SAME.

1,407,749.

Specification of Letters Patent. Patented Feb. 28, 1922.

No Drawing.

Application filed June 30, 1920. Serial No. 392,996.

To all whom it may concern:

Be it known that we, ALCAN HIRSCH and MARX HIRSCH, citizens of the United States, and residents of New York, in the county of New York and State of New York, have invented certain new and useful Improvements in Flotation Agents and Methods of Making the Same, of which the following is a specification.

10 The invention relates to improvements in ore flotation agents and method of making the same, and particularly those of the aromatic amine class. It has been customary to make an ore flotation compound by taking 15 pure naphthalene and nitrating and reducing the same to form alpha-naphthylamine and taking pure xylene and nitrating and reducing the same to form the amido substitution product thereof, and then mixing 20 the substantially pure amines to form a flotation compound commonly known as x-cake flotation reagent. It has hitherto been assumed that these materials must be made substantially pure before mixture in order to 25 get the desired results, and furthermore in the nitration and reduction of naphthalene to make naphthylamine it has been in a solid state and therefore difficult to treat and separate from the reaction material and accompanying impurities formed.

We have discovered that the usual impurities accompanying such crude aromatic compounds, and particularly the impurities accompanying crude commercial naphthalene and xylene, when subjected to the usual treatment in making the corresponding amines, do not decrease the flotation value of the naphthylamine and xylidine, but they tend rather to increase the flotation value. 40 We have furthermore discovered that great commercial advantages result from the mixing of the raw materials such as naphthalene and xylene and then nitrating and reducing the mixture to form the mixed amines, instead of nitrating and reducing them separately.

While the invention in its broader aspects is not limited to the particular aromatic amines used, nor to the particular chemical reagents used, we prefer to use a mixture of naphthylamine and xylidine prepared from crude naphthalene and xylene by the use of well known nitrating and reducing reagents. Accordingly, we set out below one 55 specific example from which those skilled in the art will understand the nature of the invention and its advantages.

Example: Take about equal parts of crude naphthalene and xylene containing the usual impurities accompanying the commercial products, and mix them together and slightly warm the mixture until they form a homogeneous fluid which may thereafter be handled substantially like benzol in the manufacture of aniline oil.

This fluid is then run in a moderate stream into a suitable commercial nitration apparatus, such as the Huff nitrator, wherein it is possible to handle conveniently and rapidly relatively large quantities of liquid material to be nitrated. For nitration mixture we prefer to use a mixed acid containing about 60% of 66° sulphuric and 40% nitric acid of 1.4 specific gravity. The temperature during nitration should preferably not rise materially above 33° C. and after the fluid mixture of crude naphthalene and xylene has all been added thereto, agitation is continued for about 2 hours to insure substantially complete reaction. The agitation is then stopped and the batch separates into layers, the nitro products containing nitro-naphthalene, nitro-xylene, some unnitrated xylene and the oxidation or nitration products of various impurities rise to the surface, and are rapidly and easily separated out by drawing off the acid from beneath.

The impurities accompanying the naphthalene and xylene may be certain phenolic oils such as carbolic acid and certain other aromatic bases such as pyridine. Owing we believe to the liquid character of the nitrated product and the presence of some unconverted xylene, the separation is easy and substantially complete. Therefore, the spent mixed acid can be readily and safely recovered and reconcentrated in the same general manner as is commonly used with spent acids used in nitrating cotton.

The fluid mixture of nitro compounds is run directly into a reducing tank in which about 1500 pounds of the nitro compound mixture are treated with about 2100 pounds of iron borings or filings in the presence of about 80 pounds of either sulphuric or hydrochloric acid, about 3000 pounds of water being added. The batch is agitated for about 2 hours and after the reduction is substantially complete as shown by the usual test for completeness of reduction, the mixture of amines and associated products is easily separated out, still as a fluid. We prefer to do this as follows: Add about 120 pounds of lime to the batch and heat the

batch to about 100° C. to neutralize the excess acid therein. The entire charge is then put into a filter press of any suitable kind, to remove the iron sludge. Water and the liquid reduction products pass out through the filter and the substantially complete removal of the liquid reduction products from the filtered cake is accomplished by blowing steam through the filter press for a short time. On standing the liquors from the filter press separate into two layers, the upper layer being a substantially acid-free mixture of the amines, alpha-naphthylamine and xylidine, and other reduction products of the impurities, not injurious to iron containers and having a very high value as an ore flotation agent, and in such a fluid form that it is very convenient to handle, pump and feed with the ore pulp, as well as to distribute and recover. The flotation material is separated from the lower layer by drawing off the lower layer, and any soluble products may be recovered by adding this lower layer to the next reduction mixture. It will be clear to those skilled in the art that other high molecular weight hydrocarbons may be used, partially or wholly, instead of the naphthalene or the xylene. In fact, in using the crude bases we do substitute in part, other materials of high molecular weight and complex, as well as of variable composition. Also other methods of forming the amine substitution products may be used. For example, nitrate of soda and sulphuric acid may be used instead of mixed acid, and the reduction may be carried out without intermediate separation of the nitration products from the acid liquor. Likewise, other neutralizing agents may be used, but we prefer lime because of its economy. Also the amount and nature of the impurities accompanying the raw materials may vary greatly. Even if it should happen that the raw bases should contain substantially no impurities, the nitration and reduction of the aromatic bases as a mixture has important advantages. Therefore, while we have described a preferred form of our improvements in great detail, we do not desire to be limited to such details or form, since many other changes and modifications may be made and the invention embodied in widely different forms without departing from the spirit and scope thereof in its broader aspects.

What we claim as new and desire to secure by Letters Patent, is:

1. A new composition for flotation of ores comprising mixed naphthalene ring and benzole ring amido substitution products accompanied by such impurities as result from the nitration and reduction of crude naphthalene and xylene.

2. A fluid composition for the flotation of

ores comprising mixed aromatic amido substitution products accompanied by impurities such as result from the formation of aromatic amines from the crude aromatic bases.

3. A composition for the flotation of ores containing a relatively large amount of an aromatic amine accompanied by such impurities as result from the nitration and reduction of the crude aromatic base to form the aromatic amine.

4. A composition for the flotation of ores comprising a mixture of naphthylamine and xylidine accompanied by such impurities as result from the nitration and reduction of crude naphthalene and crude xylene to form the amido substitution products.

5. The process of making ore flotation material, which consists in nitrating and reducing a mixture of crude benzole ring and naphthalene ring bases to form the amido substitution products thereof.

6. The process of making ore flotation material, which consists in taking a mixture of crude naphthalene and crude xylene and nitrating and reducing the mixture to form a mixture of naphthylamine and xylidine accompanied by such impurities as result from the nitration and reduction of mixed crude bases.

7. The process of making mixed amines which consists in mixing substantial quantities of a normally solid aromatic base with a normally liquid aromatic base to form a fluid mixture thereof and nitrating and reducing the fluid mixture to form the mixed amines.

8. The process of making mixed amines, which consists in forming a fluid mixture of different aromatic bases and nitrating and reducing the fluid mixture to form the mixed amines.

9. The process of making mixed amines, which consists in nitrating and reducing a mixture of benzole ring and naphthalene ring bases to form a mixture of the amido substitution products thereof, neutralizing the excess acid in the mixture and separating the aqueous liquor from the mixture.

10. The process of making an ore flotation composition which consists in taking a crude aromatic base and nitrating and reducing the same to form a flotation composition containing a relatively large amount of the aromatic amine accompanied by such impurities as result from the action of the nitrating and reducing operations on the impurities in the crude aromatic base.

Signed at New York, in the county of New York and State of New York this 29th day of June, A. D. 1920.

ALCAN HIRSCH.  
MARX HIRSCH.